

Jan. 26, 1943.

R. NEIMAN

2,309,136

PROCESS FOR PREPARING AN ALLOY FOR CAST DENTURES

Filed May 4, 1940



INVENTOR.

ROBERT NEIMAN

BY

*Joseph A. Rave*  
ATTORNEY.

## UNITED STATES PATENT OFFICE

2,309,136

PROCESS FOR PREPARING AN ALLOY  
FOR CAST DENTURES

Robert Neiman, Louisville, Ky., assignor to Edmund A. Steinbock, Louisville, Ky.

Application May 4, 1940, Serial No. 333,378

1 Claim. (Cl. 75—171)

This invention relates to a non-ferrous alloy or alloys combining high resistance to corrosion and strength, of which, the hardness and resilience can be simply and easily controlled in the melting and casting process thereof.

While this alloy is well suited for forming a wide variety of commercial articles, it is most eminently suited for producing articles by the casting process, especially dentures. Its use and advantages for the exacting nature and process of producing dentures will be described herein-after in detail.

In producing a cast alloy denture the following steps are the usual procedure:

1. An impression of the portion of the mouth containing the area to be reconstructed is taken with plaster, plastic materials, or colloidal materials.

2. A permanent cast or model of this impression is poured of dental stone.

3. An impression of the permanent cast is taken, preferably in colloidal material.

4. A casting model is poured, into this latter impression, using the investment on which the metal is to be cast this forming the lower part of the mold.

5. The desired denture is formed on this model in wax.

6. Sprues of wax are attached and the whole is encased in additional investment forming the upper part of the mold.

7. The entire mold is heated in a suitable furnace to such temperature as will eliminate the wax, and expand the mold sufficiently to counteract the casting shrinkage of the metal, and also to permit the alloy to cast successfully.

8. The mold is placed in a casting machine, the metal is melted in a crucible, usually by means of an oxyacetylene flame, and the molten alloy is forced into the cavity in the mold under pressure.

9. The mold is cooled, preferably by quenching in water, the casting is removed, cleaned and polished for use.

To produce the best possible denture with a minimum of effort or cost, the alloy, also commonly referred to as metal in the art, should have many qualities of which the following are paramountly necessary or desirable.

The metal must have good castability, that is, it must form a liquid of low viscosity when heated to casting temperature so as to flow into the fine and often minutely thin and attenuated portions of the mold. This low viscosity should be attained with a minimum amount of super-

heat between the melting point and casting temperature of the alloy so as to minimize oxidation or nitrification in the air as well as interaction with the refractory surfaces of the mold. Furthermore, the metal should not form a surface scum or slag which prevents the operator from easily seeing when the nuggets or pieces of metal are fully molten. A shiny surface on the fluid molten metal, not unlike that shown by precious metals or alloys, gives the operator an excellent chance of noticing when the metal has reached the right condition for casting.

The metal should have the property of forming castings that are homogeneous, dense, and free from pits or blowholes.

The metal should not change greatly in strength or hardness upon cooling of the mold, whether it be by quenching in water or air immediately or at any time after casting. Its casting shrinkage should be sufficiently small to enable extreme accuracy of fit of casting without resort to unusually high expanding investments, the latter being difficult to attain. The cast denture should have a surface as smooth and free of oxide and other contamination as possible, in order to reduce the time necessary for cleaning and polishing. This is most necessary on the surface in contact with the model where removal of any appreciable portion of the surface would obviously prevent accurate fit.

The metal should have a low melting point for ease in melting and a low casting shrinkage. A low casting temperature and low reactivity at this temperature are most important advantages as they enable the use of investments with calcium sulfate binders. The latter investments are the easiest to manipulate, stronger and least troublesome to use.

Corrosion resistance to a high degree is absolutely necessary. The metal should not be acted on or visibly discolored by food acid, lactic acid, or other acid, or alkalies present in foods, dentifrices, or medicinal agents. Furthermore, it should be tissue tolerant in its lack of metallic taste or other undesirable effects on the tissues, such as discomforts due to electrolysis effects with other metals present in the mouth. It should be capable of receiving a high polish and must maintain this lustre in use.

The denture must have a high strength and resilience to withstand successfully the continued subjection to stresses and strains of mastication without losing its initial shape or configuration. In addition it should have the strength and resilience necessary to permit the use of extremely

thin and narrow portions or sections. There must be an accompanying toughness and sufficient ductility to enable slight adjustments, especially of clasps, as well as to withstand overloads and occasional undue impacts. This means that the alloy should possess a high elastic limit, ultimate tensile strength, modulus of elasticity, and yet have a sufficient elongation or ductility. High values in impact and fatigue tests are also desirable. This multitude of desirable mechanical properties must not be accompanied by any appreciable brittleness nor should the hardness as measured by the Brinell test be too high. The Brinell number should be preferably within the limits of 200-300. A high Brinell number or the presence of a hard constituent would mean injury to the teeth when placing and removing the denture. This latter condition means that the alloy should be a homogeneous and preferably a single phase solid solution.

The term denture includes a variety of appliances such as partial dentures, complete dentures, inlays, crowns, and similar articles. In the construction of these varied appliances there is a necessity for using alloys of varying degrees of hardness as is known in the art. Furthermore, some dentists desire a slightly softer alloy than other in order to give them greater freedom in making adjustments of clasps, etc. It would therefore be especially desirable that the technician be able to vary the hardness of the alloy to suit these varying needs without detracting appreciably from the other desired mechanical properties. This process should preferably be performed before the denture is fitted and polished so as to preclude the necessity of double work in polishing and chance of distortion when subjected to such process as heat treatment.

The ability of the alloy to permit melting in an open crucible by such means as an oxy-acetylene flame means less cost and trouble than one requiring inert or reducing atmospheres, or special melting furnaces. The alloy should also permit soldering or welding without complicated or costly apparatus or technics.

A low specific gravity, low cost of metal and casting equipment, a warm platinum like color rather than a harsh bluish tinge of chromium, and good heat conductivity are further desirable properties.

To meet this extremely difficult host of requirements the art has found gold and alloys thereof to meet most but not all of the requirements. A number of non-ferrous, non-precious metal alloys are available that also meet most of the requirements but are usually of high melting point, require costly casting equipment, or fail to give the operator a control of the hardness characteristics.

Alloys consisting of chromium and cobalt or of these two metals in conjunction with tungsten or molybdenum, or both, have the advantage over precious alloys in their comparatively low cost and greater modulus of elasticity but their melting point is so high as to preclude the very convenient use of calcium sulfate investments. Even when alloyed with nickel, silicon, manganese, titanium or combinations therefrom the melting point is still too high. Also the hardness is generally too high and cannot be easily controlled by the operator. Ternary alloys of chromium, cobalt, and nickel also offer similar disadvantages.

The addition of beryllium or boron to the latter ternary alloys serve to reduce the melting point

but are generally somewhat brittle and not readily susceptible to hardness control by the operator.

Many other commercial alloys are available that resist corrosion well but lack one or more properties that makes them as suitable as desired. Stainless steel, such as the 18% chromium-8% nickel variety, is fairly corrosion resistant to a number of media but the high melting point precludes its castability in moulds having calcium sulfate as the binder. Another type of alloy—"Nichrome"—containing 80% nickel and 20% chromium is also too high melting and too reactive at the casting temperature, moreover, this alloy is too soft. The substitution of cobalt for all or part of the nickel increases the hardness but does not lower the melting point or reactivity at casting temperature sufficiently for use in conjunction with calcium sulfate investments.

It is, therefore, the principal object of this invention to provide an alloy or alloys that possess a comparative high degree of excellence in every one of the following desirable properties and a combination of all of them in such degree as to render the alloys admirably suited for dentures. Obviously, alloys possessing these desirable attributes are also advantages in industry for a multitude of uses.

1. Good castability.

2. Low melting point and casting temperature readily discernible.

3. Form smooth, homogeneous, dense, and blow-hole free castings.

4. Strength not greatly affected by rate of quenching.

5. A low casting shrinkage.

6. Low reactivity at casting temperature.

7. Castable in a calcium sulfate investment.

8. High corrosion resistance.

9. High elastic limit.

10. High ultimate tensile strength.

11. High modulus of elasticity.

12. High modulus of resilience.

13. Sufficient ductility to obviate brittleness.

14. High impact strength.

15. High fatigue value.

16. Desirable and controllable Brinell hardness.

17. Permit soldering and welding readily.

18. Low specific gravity.

19. Low cost of metal.

20. Low cost of melting and casting equipment.

21. Attain a high lustre readily.

22. Possess a warm platinum-like color.

23. Good heat conductivity.

24. Contain little or no high abrasive constituents.

25. Form a homogeneous and preferably a single phase solid solution.

Other objects and advantages of the present invention should be readily apparent by reference to the following specification considered in conjunction with the accompanying drawing forming a part thereof and it is to be understood that any modifications may be made in the exact details there shown and described, within the scope of the appended claim, without departing from or exceeding the spirit of the invention.

In the drawing, the figure illustrates a flame that is employed to obtain the results of this invention.

As above mentioned, cobalt-chromium-molybdenum alloys have many desirable features but are primarily of a high melting point and form solid solutions within a limited field of the ternary diagram.

Binary alloys of nickel and copper may be made in any proportions as these two metals are mutually soluble. Binary alloys of these two metals especially with high nickel content are fairly corrosion resistant but not as highly as the above ternary alloys. On the other hand, the binary alloys are not as brittle and, consequently, more ductile.

While no study has ever been made of the complete alloy system containing all five metals, we can surmise from known metallurgic principles certain facts which explain the peculiar desirable results of mixing these five metals in certain limited proportions.

When metals are at least partially soluble in each other, the addition of one metal to another results in an alloy possessing a lower melting point than that of either metal alone. The addition of two new metals to a ternary alloy will thus reduce its melting point considerably. Furthermore, the more corrosion resistant metals will impart this same property to the newer alloy as a whole. Also, the addition of the binary alloys to the above ternary system tends to form a more homogeneous metal in perhaps a greater range of compositions since there are now present more combinations of metals with mutual affinities for each other. The added nickel-copper also reduces the carbide forming tendency of the alloys as a whole since neither of these two metals form carbides readily, if at all. The binary alloys alone have a soft and pleasing color and impart this to the completed alloy. The nickel-copper addition also imparts its ductility without deteriorating the toughness of the alloys appreciably.

Of the metals mentioned above, chromium is the basis and makes this type of alloy possible. Whereas precious alloys attain their corrosion resistance through the "noble" metals present, alloys containing appreciable amounts of chromium attain theirs through the "passivity" of the surface due to the chromium present, chromium alloys become "passive" because the surface film is oxidized in the air or generally, even in aqueous solutions though they be acid, alkaline, or neutral. The oxide film formed is invisible and is between 1 and 40 molecules thick. This oxide film is so dense that it is impervious to the further diffusion of oxygen or other corrosive agents. This film is very tenacious and the prime reason for its continued protection of the metals is the fact that the film even when broken is immediately self-repairing. This is true wherever there is possible access of oxygen. Furthermore, this film has approximately the same coefficient of expansion as the metal as a quite abrupt change in temperature will not cause it to flake off. It is this "passive" oxide film that is corrosion resistant, rather than the metal itself.

Chromium is also most important from the mechanical standpoint as it imparts strength and hardness to the alloy as a whole. When used in the greater proportion within the limits specified in the table below, it will tend to harden the metal and unless there are softening metals present, the alloy as a whole while becoming more corrosion resistant will, nevertheless, lose in ductility. Chromium contents within the preferred proportions given below render the alloy tough and extremely resistant to such acids as nitric, in fact, the alloy will resist concentrated nitric acid for unlimited periods. Nitric acid is very useful in forming the "passive" surface referred to above because of its oxidizing action.

Cobalt is a grayish metal with a slight tint of red. It imparts this reddish tone to its alloys which adds warmth to their color. Cobalt also forms a protection "passive" oxide film. It is a fairly hard metal and imparts strength to the alloy and when not used in too great proportions, does not cause brittleness.

Molybdenum, when used, within the limits set forth imparts strength and acid resistance, especially to hydrochloric acid. The acid resisting property of molybdenum is believed by some to be due to the fact that it is a noble metal since it is below hydrogen in the electromotive series. In spite of its high melting point it seems to lower the melting point of the alloy.

Nickel is a strong and tenacious metal and also forms a protective oxide film. It adds toughness and ductility to the finished alloy.

Nickel may be interchanged with cobalt within the limit specified and when thus replacing cobalt, it tends to add ductility to the alloys, whereas, cobalt adds greater resilience. These two metals seem to combine their respective desirable properties when present in approximately equal proportions as given in the preferred alloys below.

Copper has a great affinity for, and solubility in nickel and renders the alloys more homogeneous and reduces the melting point. While it is not extremely acid resistant alone, it does not seem to reduce the acid resistance of the alloy since it is in solid solution and, furthermore, it also forms a protective oxide film. When using this metal, the higher proportions should preferably be used when the nickel content is also high as, otherwise, it may tend to border on the range of a two phase system.

Iron is to be kept as low as possible in order to maintain a high corrosion resistance along with other good properties possessed by these alloys. Since iron is an appreciable impurity in practically all of the constituent elements as commercially available, it will occur in the finished alloy in amounts generally between 1.0 and 2%. It can hardly be kept below 1% and in rare cases may be as high as 5%. In any case, the iron is not to be considered as a necessary alloying element, but merely as an undesirable impurity that must of necessity be tolerated.

To this combination of five elements, making up from 97% to over 99% of the alloy, it is desirable to add small amounts of certain elements to remove undesirable impurities, to prevent contamination in the melting process, and to modify and control the physical characteristics.

Silicon, in amounts of approximately .2 of 1% increases the castability by improving the fluidity. It also makes it easier for the operator to discern when the metal has reached its casting temperature by reducing the obscuring, non-metallic surface film. This small amount is more than likely entirely dissolved in the alloy and, thus, does not form hard intergranular constituents. It also seems to be effective in controlling and limiting the amount of carbon dissolved in the alloy during the melting operation and thus acts as a "brake" in preventing carbide formation.

The manganese serves to combine with the sulphur present as impurities in the other elements by forming globularized manganese sulfide which generally enters the slag or, if retained in the alloy, has no appreciable deleterious effect. If the sulphur is not thus removed, it tends to alloy with the nickel, especially. These two elements form a very low melting eutectic that coats the

surface of the grains of the alloy and renders the latter extremely weak and brittle.

Carbon, perhaps of all the elements, has the unusual property of not only hardening these alloys but of giving them a springiness or resilience combined with toughness, when present in small amounts. This is very likely true so long as the carbon is dissolved in the alloy. Once an excess of carbon is present, it begins to form carbides, which cause embrittlement of the alloy. Furthermore, carbides are undesirable as they are very abrasive and would injure the teeth when the denture is removed and replaced. The alloys herein given, especially the preferred ones, have been found to absorb the desired amount of carbon when melted by the method hereinafter described. Furthermore, when melted by different operators there seems to be but a negligible variation in carbon absorption provided a given flame is used.

The carbon in the original alloy should be low—preferably under 0.20% and may be added to in the melting process herein described up to approximately 1.0%. Alloys with less than 0.2% carbon may be referred to as practically carbon free alloys.

The melting process in which the carbon is imparted to the alloy in controlled amounts is performed as follows:

The equipment consists of a tank of oxygen, a tank of acetylene, each equipped with regulating gauges and connected by a suitable tubing to the torch. A torch made by the Imperial Brass Manufacturing Co., of Chicago, Ill., and using Tip #8 has been found very successful. Substantially, similar torches may be secured from many manufacturers, especially those dealing in the two gases mentioned above.

To adjust the flame, the following procedure is used:

1. Close both valves on torch.
2. Open valves on oxygen and acetylene tanks fully.
3. Set regulator gauge valve for acetylene at 5 lbs. "flow pressure," by opening the acetylene torch valve when adjusting the gauge.
4. Set regulator gauge valve for oxygen at 10 lbs. "flow pressure," by opening the oxygen torch valve when adjusting the gauge.
5. Light torch.
6. With the acetylene torch valve fully opened, giving 5 lbs. "flow pressure," adjust the oxygen flow by means of its torch valve until the flame is as shown in Figure 1. The inner oxidizing cone 10 will be  $\frac{3}{4}$  inch to 1 inch long the reducing cone 11 will be approximately  $2\frac{1}{2}$  inches long. It is important that the flame, that is, the sum of the oxidizing and reducing cones, should measure  $3\frac{1}{2}$  inches long from the edge of the tip.

7. The nuggets of metal are melted by impinging this flame in such manner that the reducing cone only is in contact with the metal. It is preferable to have the center of this cone, that is, the portion of the flame between 2 and  $2\frac{1}{2}$  inches from the edge of the tip, in contact with the metal.

The above flame is known as a  $3\frac{1}{2}$  inch flame and is the one generally preferred for use with the "preferred" alloy.

To harden the alloy, the flame may be increased in length to 4 inches, for example. To soften the alloy the flame is decreased to 3 inches or even less. Increasing the flame length imparts more carbon to the alloy, thus hardening it, whereas decreasing the flame length imparts less carbon and thus the alloy remains more ductile.

As a concrete example—an alloy made about midway between the preferred alloy limits shown in the table, contained but 0.15% carbon. It showed a Brinell hardness (BHN) of 150 (500 kg. load) and a Rockwell "C" (Rc) hardness of 20-22.

When  $1\frac{1}{2}$  oz. were molten and cast with a 2" flame, the carbon was increased to 0.25% and the BHN was 109, Rc was 12-14. Thus, even though the carbon was increased, the hardness was reduced. This is explained by the fact that the size, shape, heat, and mechanical treatment of the test pieces were different.

Using a  $3\frac{1}{2}$ " flame the carbon was increased to about 0.5%, the BHN was 130, Rc 21 to 23.

15 The use of a still longer and more reducing flame, one of  $4\frac{1}{4}$ ", the carbon was increased to about 0.6% and the BHN was 143, Rc 21 to 22.

The test pieces for the tests, other than the original alloy were cast under practical conditions and show that the carbon and BHN are increased as the flame is made longer and more reducing. The Rc is also increased but not in exact ratio.

20 It is interesting to note that it is apparently impossible to exactly correlate the BHN and the Rc. This is very likely associated with the work hardening of these alloys. It is further interesting to note that whereas the Rc hardness indicates that the alloys are soft enough to machine, it is, nevertheless, practically impossible to mill or file specimens without damaging the milling cutter and the file. For this reason, and also due to the fact that specimens when cast in small and thin pieces comparable to the size of dentures, it was undesirable to use the 3,000 kg. load Brinell 25 hardness test. The 3,000 kg. BHN would be about twice the BHN (500 kg. load) and, therefore, range between 200 and 300 as is most desirable for the intended uses.

The castings on which tests were made were 30 cast in a mold having a calcium sulfate binder, the investment mold having been raised to 1600° F. in about  $1\frac{1}{2}$  hrs. and maintained at this temperature for 1 hour. The properties of the alloys are variable somewhat depending on the mold 35 temperature as this determines the rate of solidification. In general a smoother and perhaps a little harder casting will result when cast at lower temperatures and a slightly rougher and more ductile casting will result at higher mold temperatures but greater detail is possible. The 40 more inert and the less possible contaminating agents present in the mold at casting temperature the smoother and more resilient the casting.

The ability to work harden is further desirable 45 in cases where clasps are to be adjusted. The metal "as cast" is readily adjustable and then, in use is hardened further and thus given a greater resilience. The ability to work harden further makes possible the drawing of the alloy into wires, etc. Thus, clasps may be made of wires and attached to the denture by soldering, welding, or casting the denture to the embedded clasp. Other commercial uses wherein work hardening is necessary or desirable is also possible.

50 Within the minimum and maximum ranges of the metals forming the alloy, it is possible to increase the carbon absorbing elements (chromium and molybdenum), or the cobalt and give the alloy sufficient inherent hardness to permit the use of even a neutral flame, that is, a flame without the center reducing cone. In this case, however, it will be found that in melting the alloy, an undesirable opaque film will cover the molten metal 55 and obscure the operator's view in adjudging the

readiness of the metal for casting by its fluidity or viscosity.

In this case, or even when flames up to approximately 3 inches in length are used, it is highly beneficial to apply a "finishing" flame. To do this, the metal is heated by the desired flame until the nuggets have slumped and the alloy appears to be completely molten, the oxygen torch valve is then closed slightly, without moving the torch, to provide about a 3½ inch to 4 inch flame. With this reducing flame, the metal is given a sufficient super-heat, from just above the melting point to the casting temperature, to enable successful casting. By using this "finishing" reducing flame, the opaque film of oxides is reduced and the surface appears shiny and readily indicates the fluidity or viscosity of the metal by the mobility and spinning action produced under the force of the impinging flame gases. This "finishing" flame length cannot be accurately adjusted since it is undesirable to remove the flame from the metal even momentarily, as this will permit the rapid oxidation and possibly solidification of the alloy. The inaccuracy of the "finish" flame length is not deleterious as its action lasts for perhaps only 10 seconds and during this short interval very little carbon is imparted to the alloy, since a great portion of it is used up in reducing the oxide film. By this means, the alloys provided herein may be easily molten and yet retained almost carbon-free.

The use of the "finishing" flame is believed to be an entirely new and novel process.

If the more ductile elements—nickel or copper, or both are used in maximum quantities herein set forth, it will be advisable to use a more reducing flame, such as, a 4" or even slightly longer, to provide the alloy with sufficient strength and resilience.

It is thus possible for a manufacturer to provide a single substantially carbon-free alloy and the user in turn can impart to this alloy a desired resilience and hardness within wide limits. Obviously, the manufacturer may add sufficient carbon to the alloy in the manufacturing process to give a desired hardness when used with a given flame length; the user still can vary the properties, should he desire, by changing the flame length. For those who desire a hard metal not requiring appreciable carbon the manufacturer may increase the chromium, cobalt, or molybdenum, or any combination of these and furnish an alloy that is very satisfactory when molten with a short flame and thence a "finishing" flame.

The alloys described and explained herein are to be considered as consisting of five metals, namely, cobalt, chromium, molybdenum, nickel, and copper; to this combination it is most desirable to add some amounts of silicon, manganese, and carbon. While the latter three elements are highly desirable, it is, nevertheless, possible to produce satisfactory alloys by omitting one or more of them. Instead of manganese it is possible to use an alloy of manganese and titanium or possibly titanium alone. It is possible to omit the silicon entirely, likewise, it is possible to adjust the five metals in such combination as to obviate the necessity for carbon. The elements silicon, manganese, and carbon are not positively essential but highly desirable if full advantage of the benefits provided by the alloys and processes given herein are to be utilized to the best possible advantage as herein provided.

Following is shown a table giving the elements that go to make up the alloys:

| Element or metal | Minimum  | Maximum  | Preferred |
|------------------|----------|----------|-----------|
|                  | Per cent | Per cent | Per cent  |
| Cobalt.....      | 18.0     | 40.0     | 30. -35.  |
| Chromium.....    | 18.0     | 28.0     | 20. -25.  |
| Molybdenum.....  | 4.0      | 12.0     | 6. -10.   |
| Nickel.....      | 19.0     | 40.0     | 30. -35.  |
| Copper.....      | 1.0      | 10.0     | 3. - 5.   |
| Silicon.....     | 0.2      | 1.0      | 0.3 - 0.7 |
| Manganese.....   | 0.1      | 1.0      | 0.1 - 0.4 |
| Carbon.....      | 0.1      | 1.0      | 0.2 - 0.7 |

While the above list gives minimum and maximum percentages by weight of each metal it is, of course, recommended to steer clear of extremes. The extreme on one metal is not necessarily undesirable, but the extreme on two or more metals is generally undesirable. Insofar as possible, the above list obviates such practices; for example, the total of the minimums on cobalt plus chromium, plus molybdenum is 40% and the total of maximums on nickel plus copper is 50%, the five elements adding up to only 90%; obviously the lower limit of the ternary combination must add up to at least 50%.

To get the best possible results, it is desirable to take a middle course on all elements and this is given in the column entitled, "Preferred"; even in this column, the middle course is a further improvement.

The preferred alloys are thus best suited and the best results attained from use with a carbonizing flame, preferably one as shown in Figure 1, namely, of 3½ inch length.

By way of further illustration and recommendation: the preferred nickel plus copper percentages of 33% to 38% limits the cobalt-chromium-molybdenum total to 62% to 67%, thus only one element of the latter three could be used in minimum quantities. The percentages given are thus, to a great extent, self-limiting.

It has been further found that certain groups of elements act very much as one element in their functions. Chromium plus molybdenum are the hardening elements and also most active in resisting corrosion. Such combination of the two as to make up approximately 30% of the alloy seems to give the best combination of high strength and moderate hardness which, in reality, is a definition of toughness. Nickel and cobalt form solid solutions in all proportions and it is possible to interchange these to a great extent, cobalt lending hardness and nickel lending ductility—a superior combination is attained with approximately equal quantities of each. Nickel plus copper are also mutually soluble in all proportions and seem to give the best results when present in the ratio of nickel to copper of between 7 and 10 to 1. Chromium and molybdenum are quite soluble in nickel although they do not form solid solutions in all proportions. It is thus seen that each of the elements has a good solubility and forms solid solutions with nickel. It is thus apparent that this summation of inter-related affinities conveys to the completed alloy an extreme homogeneity that combines the good characteristics of each constituent to the best possible advantage. Furthermore, the above also explains why the five metals mentioned form solid solutions within wide ranges of composition.

In the matter of minor elements, namely, silicon, manganese and carbon a medium course in composition is also of advantage. In the preferred alloy all three elements make up approxi-

mately 1.5% of the total. In manufacturing these alloys it is desirable that they be melted in an induction furnace and preferably also in a carbon-free crucible. The alloy should be melted under a glass slag to prevent undue reaction with gases in the air, especially oxygen. This slag is desirable although not absolutely necessary.

Once the alloy is molten it should be cast or poured, into a refractory, or preferably a metal mold, into the form of rods which can then be cut or broken into small pieces suitable for convenient use. If the pieces are appreciably contaminated on the surface, they should be cleaned by sandblasting or tumbling.

The original alloy made for use should be as 15 carbon-free as possible since even small amounts may be deleterious, not necessarily alone, but when additional carbon is absorbed in the melting process just prior to casting. Wherever it is desirable to make the original alloy with a given amount of carbon so that a shorter flame may be used in melting, it is possible to use a furnace or crucible containing carbon or graphite. This has been found generally to be inferior to the use of an induction furnace.

The use of small amounts of various elements which function as fluxes and remove impurities in the original metals is possible. For example, calcium is a very powerful de-oxidizer and may be used in small amounts. Similar metals, such as zirconium or titanium, the latter also a powerful dentrifier, may also be used as fluxes, so long as they do not appear in the finished alloy in amounts sufficient to act deleteriously.

5 The use of the oxy-acetylene flame has been herein described in detail and is generally the preferred form for melting the alloy just prior to casting. It is, however, possible to melt the metal with other gas flame combinations and, also, to melt it by using electricity as the source of heat. In the latter cases it is desirable to adjust the carbon in the original alloy so that the final casting 10 will contain the desired amount of carbon and be within the recommended limits of .1 to 1%. Carbon may also be added to the metal by melting it in contact with carbon.

15 What is claimed is:

The process of preparing an alloy to make a cast denture in a mold containing a calcium sulfate binder, and said alloy consisting of cobalt 18 to 40%, chromium 18 to 28%, molybdenum 4 to 12%, nickel 19 to 40%, copper 1 to 10%, silicon .2 to 1%, manganese .1 to 1%, and carbon .1 to 20 1%, and including the steps of melting the alloy with a substantially neutral flame, in which the reducing cone is short or entirely absent, and following with a finishing flame, in which the reducing cone is increased in length to provide a 25 reducing condition, whereby the surface oxide film of the alloy is substantially removed, thus improving the visible condition of the molten alloy, and which finishing flame is not used for a sufficient length of time to impart any appreciable amount of carbon to the molten alloy.

30 ROBERT NEIMAN.